

## UNITED STATES PATENT OFFICE

2,040,797

## ALLOY CONTAINING COPPER AND PHOSPHORUS

Georg Sachs and Arthur Burkhardt, Frankfort-on-the-Main, Germany, assignors to American Lurgi Corporation, New York, N. Y., a corporation of New York

No Drawing. Application January 5, 1932, Serial No. 584,906. In Germany January 9, 1931

2 Claims. (Cl. 148—32)

It is a known fact, that compounds of metals with metalloids, such as for example phosphides, silicides, carbides and antimonides in the cast condition are brittle to a high degree. The brittleness is such, that the compounds cannot even be scratched without breaking into splinters. This brittleness is exhibited also to a great extent by alloys containing an appreciable percentage of such compounds. If for example copper contains 5 a high percentage of copper phosphide, it is so brittle that it can be crushed by trifling shocks. On the other hand compounds of metals and metalloids, and alloys containing them in a high percentage, possess a number of very valuable 10 properties, such as great hardness, resistance against corrosion, etc. However the utilization of these good qualities has hitherto been handicapped, because the mechanical working of such material has been considered to be impossible.

20 The object of the present invention is the preparation of alloys comprising a predominating proportion of copper and more than 6% of phosphorus, which alloys possess greatly improved mechanical properties in comparison with hitherto known alloys of the same composition. Because 25 of their increased strength and increased stability they are useful for the manufacture of utensils and tools. The process of improving these mechanical properties consists in mechanically 30 straining or thoroughly kneading at elevated temperatures, i. e. temperatures closely below the melting point of the alloy. By such a treatment particularly the strength of these alloys is increased to an extraordinary extent. Moreover by 35 thoroughly kneading once or several times at an elevated temperature a kind of ductilization is attained, so that these alloys may be subsequently strained even at low temperatures. There are already known methods by which certain pure 40 metals which are brittle after having been cast, such as tungsten, or chromium, are rendered ductile by hammering. It was however hitherto unknown, that also copper alloys containing a relatively high proportion of phosphorus could 45 be improved in regard to their ductility by mechanical strain, for instance by pressure at a higher temperature. By ductilization, is meant that by raising the temperature to above a critical point the ductility of the material is increased 50 to such an extent that straining at high temperatures is possible. Moreover by a single thorough kneading at a temperature closely below the melting point, such a permanent improvement of the ductility of the material is attained that a further 55 straining at lower temperatures, even in the cold,

is possible without splintering the material or without making chips.

Copper with contents of more than 6% P was heretofore considered not to be rollable either hot or cold. The invention, therefore, refers to such 5 compounds of copper with phosphorus either in the pure state or in the form of alloys containing more than 40% by weight thereof.

It has been found for instance, that copper phosphide containing more than 6% P may be 10 rendered mechanically treatable, at a temperature closely below the melting point. The melting point of the eutectic is about 707° C. When copper phosphide containing more than 6% P is strained at temperatures between about 650 and 15 700° C., the material is rendered plastic.

It is however highly surprising, that the material treated in this manner can be rolled out to any desired thickness within a fairly wide range of temperatures, for instance between 400 and 20 600° C. i. e. the plasticity of the material is then permanent. With higher contents of phosphorus, for example 10% P, a more intensive preliminary mechanical treatment at the critical temperatures is required, i. e. the material has to be subjected 25 to pressure before it can be rolled down to a desired thickness. In this manner even phosphides containing up to 13% P may be rolled into thin sheets.

The kneading of the material is preceded by an 30 application of pressure at temperatures of about 30 to 100° C. below the solidus-point, whereupon they may undergo any desired further mechanical straining. The further straining may of course be omitted, if the finally desired shape of the work 35 piece can be attained by pressure alone.

Besides the pure copper-phosphorus alloys, the process according to the invention naturally may also be applied to all alloys containing more than 40% of copper phosphide.

40 So by the invention the possibility arises of utilizing materials hitherto rejected as being useless, for quite a number of technical purposes. There may, for example, be particularly mentioned a copper alloy containing about 8% phosphorus, suitable for welding, because such copper phosphide may now be brought into the form of wire or rods by pressure, thus facilitating its employment in practical use.

50 We claim:

1. An alloy containing a predominating proportion of copper and more than 6% but not more than 14% of phosphorus which alloy has been plastically deformed at a temperature closely below its melting point whereby its mechanical 55

properties are improved and its strength increased and which is capable of being strained at low temperatures without splintering.

- 5 2. An alloy containing a predominating proportion of copper and more than 6% but not more than 14% of phosphorous, which alloys has been plastically deformed at a temperature of 650° C.

to 700° C. whereby its mechanical properties are improved and its strength increased and which is capable of being strained at lower temperatures without splintering.

GEORG SACHS.  
ARTHUR BURKHARDT.